

# United States Patent Office

2,981,621

Patented Apr. 25, 1961

1

2,981,621

## HIGH TEMPERATURE NICKEL-IRON BASE ALLOY

Rudolf H. Thielemann, Palo Alto, Calif., assignor to  
Sierra Metals Corporation, a corporation of Delaware

No Drawing. Filed July 29, 1957, Ser. No. 674,568

10 Claims. (Cl. 75—171)

This invention relates to an iron-nickel base austenitic type metal alloy, and particularly to one such alloy which includes chromium and tungsten, as well as other constituents.

Important features of the iron-nickel base austenitic metal alloy are (1) it possesses high strength at elevated temperatures of the order of 1200° F. to 1500° F.; (2) is readily forgeable at temperatures in the range of from 1950° F. to 2100° F.; (3) is corrosion resistant at temperatures of from 1200° F. to 1500° F.; and (4) is capable of withstanding thermal shock.

As a result of these markedly improved, superior high temperature properties, the metal alloy of this invention is particularly useful as a wheel (1) in an aircraft gas turbine engine and (2) in a high pressure steam turbine, as well as the material for other parts in all types of engines, such as valve seats, exhaust valves, and the like.

The prior art iron base metal alloys used as wheel material in aircraft gas turbine engines, such as A-286 (14.5 percent of chromium, 26 percent of nickel, 1.25 percent of molybdenum, 2 percent of titanium, 0.3 percent of vanadium, and the balance, essentially iron), are, for all practical purposes, non-utilizable at temperatures of 1200° F. and above since the strength characteristics thereof are too low for use as wheel material at such elevated temperatures. In contrast, the alloy of this invention maintains its strength characteristics at temperatures up to 1500° F., as do also wheels made from this alloy and used in gas turbine engines which wheels are subject to temperatures between 1200° F. and 1500° F.

The iron-nickel base metal alloy of this invention is comprised, by weight of approximately: 10 to 20 percent of chromium, 18 to 50 percent of nickel, 1.5 to 8 percent of tungsten, 1 to 5 percent of columbium, or tantalum, or mixtures thereof, 2 to 4 percent of titanium, 0.05 to 0.25 percent of carbon, and the balance, essentially iron.

To achieve the optimum desired properties, the following impurities preferably should be held to the following limits by weight in the alloy. The manganese content in the final alloy should be no more than about 2.0 percent, the silicon content, no more than about 1.0 percent, and the aluminum content, no more than about 0.5 percent.

As will be seen from the examples herein, the strength characteristics at elevated temperatures of the alloy of this invention are improved by the addition of cobalt. I have found that the addition of cobalt in amounts up to 10 percent by weight of the final alloy, preferably 1 to 10 percent by weight of cobalt, imparts to the alloy the desired strengthening effect.

I have further found that small additions of both boron and zirconium greatly improve the hot workability of the metal alloy of this invention and markedly reduces the amount of cracking which occurs during forging of ingots made from the alloy. In addition, these two constituents improve the high temperature metallurgical stability and strength characteristics of the alloy of this invention.

It is important to note that the maximum amount of boron which may be used in the alloy of this invention is

2

about 0.1 percent and the maximum amount of zirconium, about 0.3 percent. If the boron or zirconium content exceeds these maximum limits, then the alloy of this invention will crack upon being hot worked and is, for all practical purposes, non-utilizable.

The following are examples of the preparation and test results of the iron-nickel base alloy of this invention.

### Example 1

10 A 5 pound ingot of an iron-nickel base metal alloy composition containing 15 percent of chromium, 27.5 percent of nickel, 3 percent of tungsten, 3 percent of titanium, 3 percent of columbium, 0.1 percent of carbon, and the balance, essentially iron, all by weight, was prepared by melting the iron under a vacuum condition of about 10 microns at a temperature of about 2900° F. and maintaining the iron in a molten condition at this temperature until degassing was complete. Nickel in an amount of 27.5 percent of the total weight of the alloy was then added, followed by 15 percent of chromium, 3 percent of tungsten, 3 percent of columbium, 3 percent of titanium, and 0.1 percent of carbon in the form of graphite. The resulting molten metal alloy was cast into an ingot mold and allowed to solidify under vacuum.

15 It is to be noted that the carbon may be added to the molten mix in the form of columbium carbide or be present in the iron.

20 Test bars (1/4 inch diameter and 3 inches long) were fabricated from this ingot by the usual hot working procedure, i.e. forging, at a temperature of between 1950° F. and 2050° F. and then heat treated in air as follows: The test bars were heated to a temperature of about 2000° F., held at this temperature for about 2 hours, cooled in air to room temperature, heated to a temperature of about 1350° F., held at this temperature for about 16 hours, and then air cooled to room temperature.

25 The fabricated, heat treated test bars had a yield strength at 0.2 percent offset of (i) 141,000 p.s.i. at room temperature, and (ii) 115,000 p.s.i. at a temperature of about 1300° F.

30 At a temperature of about 1300° F. in air and under a load of 70,000 p.s.i., the rupture life of these test bars was in excess of 100 hours.

### Example 2

35 A 5 pound ingot of an iron-nickel base metal alloy composition containing 15 percent of chromium, 27.5 percent of nickel, 3 percent of tungsten, 3 percent of titanium, 3 percent of columbium, 5 percent of cobalt, 0.1 percent of carbon, and the balance, essentially iron, all by weight, was prepared in the same manner as set forth in Example 1, with the exception that the 5 percent of cobalt was added to the iron melt in addition to the constituents of the alloy of Example 1.

40 Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 150,000 p.s.i. at room temperature and (ii) 125,000 p.s.i. at a temperature of about 1300° F.

45 At a temperature of about 1300° F. in air and under a load of 70,000 p.s.i., the rupture life of these bars was in excess of 100 hours.

### Example 3

50 A 5 pound ingot of an iron-nickel base metal alloy composition containing 15 percent of chromium, 27.5 percent of nickel, 3 percent of tungsten, 3 percent of titanium, 3 percent of columbium, 5 percent of cobalt, 0.2 percent of zirconium, 0.015 percent of boron, 0.1 percent of carbon, and the balance, essentially iron, all by

weight, was prepared in the same manner as set forth in Example 1, with the exception that the above proportions of cobalt, zirconium and boron were added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 150,000 p.s.i. at room temperature and (ii) 125,000 p.s.i. at a temperature of about 1300° F.

At a temperature of about 1300° F. in air and under a load of 70,000 p.s.i., the rupture life of the test bars of this example was in excess of 100 hours.

The workability of the test bars of this example was much better than the workability of the test bars of Examples 1 and 2. This is due to the incorporation of zirconium and boron in the alloy of this example.

#### Example 4

A 5 pound ingot of an iron-nickel base metal alloy composition containing 10 percent of chromium, 18 percent of nickel, 1.5 percent of tungsten, 4 percent of titanium, 1 percent of tantalum, 0.25 percent of carbon, and the balance, essentially iron, all by weight, was prepared in the same manner as set forth in Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 140,000 p.s.i. at room temperature and (ii) 113,000 p.s.i. at a temperature of about 1300° F.

The rupture life of the test bars of this example was in excess of 100 hours when subjected to a temperature of about 1300° F. in air and under a load of 70,000 p.s.i.

#### Example 5

A 5 pound ingot of an iron-nickel base metal alloy composition containing 10 percent of chromium, 18 percent of nickel, 1.5 percent of tungsten, 4 percent of titanium, 1 percent of columbium, 10 percent of cobalt, 0.1 percent of carbon, and the balance, essentially iron, all by weight, was prepared in the same manner as set forth in Example 1, with the exception that the 10 percent of cobalt was added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 145,000 p.s.i. at room temperature and (ii) 122,000 p.s.i. at a temperature of about 1300° F.

At a temperature of about 1300° F. in air and under a load of 70,000 p.s.i., the rupture life of these test bars was in excess of 100 hours.

#### Example 6

A 5 pound ingot of an iron-nickel base metal alloy composition containing 10 percent of chromium, 18 percent of nickel, 1.5 percent of tungsten, 4 percent of titanium, 1 percent of columbium, 5 percent of cobalt, 0.2 percent of zirconium, 0.015 percent of boron, 0.1 percent of carbon, and the balance, essentially iron, all by weight, was prepared in the same manner as set forth in Example 1, with the exception that the above proportions of cobalt, zirconium and boron were added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had

a yield strength at 0.2 percent offset of (i) 148,000 p.s.i. at room temperature and (ii) 125,000 p.s.i. at a temperature of about 1300° F.

The rupture life of these test bars at a temperature of about 1300° F. in air and under a load of 70,000 p.s.i. was in excess of 100 hours.

#### Example 7

A 5 pound ingot of an iron-nickel base metal alloy composition containing 10 percent of chromium, 50 percent of nickel, 8 percent of tungsten, 3.5 percent of titanium, 5 percent of columbium, 0.1 percent carbon, and the balance, essentially iron, all by weight, was prepared in the same manner as set forth in Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 152,000 p.s.i. at room temperature and (ii) 127,000 p.s.i. at a temperature of about 1300° F.

At a temperature of about 1300° F. in air and under a load of 65,000 p.s.i., the rupture life of these test bars was in excess of 100 hours.

#### Example 8

A 5 pound ingot of an iron-nickel base metal alloy composition containing 10 percent of chromium, 50 percent of nickel, 8 percent of tungsten, 3.5 percent of titanium, 5 percent of tantalum, 5 percent of cobalt, 0.1 percent of carbon, and the balance, essentially iron, all by weight, was prepared in the same manner as set forth in Example 1, with the exception that the 5 percent of cobalt was added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 156,000 p.s.i. at room temperature and (ii) 129,000 at a temperature of about 1300° F.

The rupture life of these test bars at a temperature of about 1300° F. in air and under a load of 70,000 p.s.i. was in excess of 100 hours.

#### Example 9

A 5 pound ingot of an iron-nickel base metal alloy composition containing 10 percent of chromium, 50 percent of nickel, 8 percent of tungsten, 3.5 percent of titanium, 5 percent of columbium, 5 percent of cobalt, 0.2 percent of zirconium, 0.015 percent of boron, 0.1 percent of carbon, and the balance, essentially iron, all by weight, was prepared in the same manner as set forth in Example 1, with the exception that the above proportions of cobalt, zirconium and boron were added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 156,000 p.s.i. at room temperature and (ii) 130,000 p.s.i. at a temperature of about 1300° F.

The rupture life of these test bars at a temperature of about 1300° F. in air under a load of 70,000 p.s.i. was in excess of 100 hours.

#### Example 10

A 5 pound ingot of an iron-nickel base metal alloy composition containing 15 percent of chromium, 27.5 percent of nickel, 3 percent of tungsten, 3 percent of titanium, 3 percent of columbium, 1 percent of cobalt, 0.2 percent of carbon, and the balance, essentially iron,

all by weight, was prepared in the same manner as set forth in Example 1, with the exception that the 1 percent of cobalt was added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 142,000 p.s.i. at room temperature and (ii) 117,000 p.s.i. at a temperature of about 1300° F.

The rupture life of these test bars at a temperature of about 1300° F. in air under a load of 70,000 p.s.i. was in excess of 100 hours.

#### Example 11

A 5 pound ingot of an iron-nickel base metal alloy composition containing 15 percent of chromium, 27.5 percent of nickel, 3 percent of tungsten, 2 percent of titanium, 3 percent of tantalum, 5 percent of cobalt, 0.3 percent of zirconium, 0.1 percent of boron, 0.05 percent of carbon, and the balance, essentially iron, all by weight, was prepared in the same manner as set forth in Example 1, with the exception that the above proportions of cobalt, zirconium and boron were added to the iron melt in addition to the constituents of the alloy of Example 1.

Test bars (1/4 inch diameter and 3 inches long) were fabricated from the ingot of this example and heat treated in the same manner as set forth in Example 1. The fabricated, heat treated test bars of this example had a yield strength at 0.2 percent offset of (i) 152,000 p.s.i. at room temperature and (ii) 127,000 p.s.i. at a temperature of about 1300° F.

The rupture life of these test bars at a temperature of about 1300° F. in air under a load of 70,000 p.s.i. was in excess of 100 hours.

#### Example 12

A 5 pound ingot of an iron-nickel base metal alloy composition containing 15 percent of chromium, 27.5 percent of nickel, 3 percent of tungsten, 3 percent of titanium, 3 percent of columbium, 5 percent of cobalt, 0.4 percent of zirconium, 0.015 percent of boron, 0.1 percent of carbon, and the balance, essentially iron, all by weight, was prepared in the same manner as set forth in Example 1, with the exception that the above proportions of cobalt, zirconium and boron were added to the iron melt in addition to the constituents of Example 1.

In attempting to fabricate test bars 1/4 inch diameter and 3 inches long from the ingot of this example, the bars cracked and could not be worked under hot working conditions.

The above detailed description of this invention has been given for clearness of understanding only. No unnecessary limitations should be understood therefrom, as modifications will be obvious to those skilled in the art.

I claim:

1. A metal alloy consisting essentially of, by weight: 10 to 20 percent chromium; 18 to 50 percent nickel; 1.5 to 8 percent tungsten; 1 to 5 percent of a metal of the class consisting of columbium, tantalum and mixtures thereof; 2 to 4 percent titanium; 0.05 to 0.25 percent carbon; and the balance, iron.

2. A metal alloy consisting essentially of, by weight: 10 to 20 percent chromium; 18 to 50 percent nickel; 1.5 to 8 percent tungsten; 1 to 5 percent columbium; 2 to 4 percent titanium; 0.05 to 0.25 percent carbon; and the balance, iron.

3. A metal alloy consisting essentially of, by weight: 10 to 20 percent chromium; 18 to 50 percent nickel; 1.5 to 8 percent tungsten; 1 to 5 percent tantalum; 2 to 4 percent titanium; 0.05 to 0.25 percent carbon; and the balance, iron.

4. A metal alloy consisting essentially of, by weight: 10 to 20 percent chromium; 18 to 50 percent nickel; 1.5 to 8 percent tungsten; 1 to 5 percent of a metal of the class consisting of columbium, tantalum and mixtures thereof; 2 to 4 percent titanium; 0.05 to 0.25 percent carbon; cobalt in an amount up to 10 percent; and the balance, iron.

5. A metal alloy consisting essentially of, by weight: 10 to 20 percent chromium; 18 to 50 percent nickel; 1.5 to 8 percent tungsten; 1 to 5 percent of a metal of the class consisting of columbium, tantalum and mixtures thereof; 2 to 4 percent titanium; 0.05 to 0.25 percent carbon; boron in an amount up to 0.1 percent; zirconium in an amount up to 0.3 percent; and the balance, iron.

15 6. A metal alloy consisting essentially of, by weight: 10 to 20 percent chromium; 18 to 50 percent nickel; 1.5 to 8 percent tungsten; 1 to 5 percent of a metal of the class consisting of columbium, tantalum and mixtures thereof; 2 to 4 percent titanium; 0.05 to 0.25 percent carbon; cobalt in an amount up to 10 percent; boron in an amount up to 0.1 percent; zirconium in an amount up to 0.3 percent; and the balance, iron.

7. A metal alloy consisting essentially of, by weight: 10 to 20 percent chromium; 18 to 50 percent nickel; 1.5 to 8 percent tungsten; 1 to 5 percent columbium; 2 to 4 percent titanium; 0.05 to 0.25 percent carbon; cobalt in an amount up to 10 percent; boron in an amount up to 0.1 percent; zirconium in an amount up to 0.3 percent; and the balance, iron.

25 8. A metal alloy consisting essentially of, by weight: 10 to 20 percent chromium; 18 to 50 percent nickel; 1.5 to 8 percent tungsten; 1 to 5 percent tantalum; 2 to 4 percent titanium; 0.05 to 0.25 percent carbon; cobalt in an amount up to 10 percent; boron in an amount up to 0.1 percent; zirconium in an amount up to 0.3 percent; and the balance, iron.

30 9. A metal alloy consisting essentially of, by weight: 15 percent chromium; 27.5 percent nickel; 3 percent tungsten; 3 percent titanium; 3 percent of a metal of the class consisting of columbium, tantalum and mixtures thereof; 0.1 percent carbon; 5 percent cobalt; and the balance, iron.

10. A metal alloy consisting essentially of, by weight: 15 percent chromium; 27.5 percent nickel; 3 percent tungsten; 3 percent titanium; 3 percent of a metal of the class consisting of columbium, tantalum and mixtures thereof; 0.1 percent carbon; 5 percent cobalt; 0.015 percent boron; 0.2 percent zirconium; and the balance, iron.

#### References Cited in the file of this patent

##### UNITED STATES PATENTS

|           |               |               |
|-----------|---------------|---------------|
| 2,432,619 | Franks et al. | Dec. 16, 1947 |
| 2,460,817 | Fisher        | Feb. 8, 1949  |
| 2,513,467 | Franks et al. | July 4, 1950  |
| 2,513,469 | Franks et al. | July 4, 1950  |
| 2,519,406 | Scott et al.  | Aug. 22, 1950 |
| 2,587,275 | Bash          | Feb. 26, 1952 |
| 2,590,835 | Kirkby et al. | Apr. 1, 1952  |
| 2,704,250 | Payson        | Mar. 15, 1955 |
| 2,742,356 | Prasse et al. | Apr. 17, 1956 |
| 2,777,766 | Binder        | Jan. 15, 1957 |

##### FOREIGN PATENTS

|            |               |               |
|------------|---------------|---------------|
| 65 785,271 | Great Britain | Oct. 23, 1957 |
|------------|---------------|---------------|

##### OTHER REFERENCES

"Effects of Columbium in Chromium-Nickel Steels," Becket and Franks, Trans. AIME, volume 113, 1934. Preprint.

ASM Preprint, 1946. "The Development of a Turbo-supercharger Bucket Alloy," Epremian. Pages 2 and 8 of specific interest.

ASM Preprint, No. 33, 1956, Salvaggi et al. Pages 8 and 9 of specific interest.